

# United States Patent

[11] 3,607,277

[72] Inventors **Karl-Wilhelm Schranz**  
Opladen;  
**Erwin Schon, Leverkusen, both of**  
Germany  
[21] Appl. No. **764,305**  
[22] Filed **Oct. 1, 1968**  
[45] Patented **Sept. 21, 1971**  
[73] Assignee **Afgo-Gevaert Aktiengesellschaft**  
Leverkusen, Germany  
[32] Priority **Oct. 14, 1967**  
[33] Germany  
[31] **P 15 97 489.7**

[56] **References Cited**  
UNITED STATES PATENTS  
3,189,452 6/1965 Pard..... 96/56 X  
3,293,036 12/1966 Meckl..... 96/60  
FOREIGN PATENTS  
739,202 10/1955 Great Britain..... 96/60  
*Primary Examiner*—William D. Martin  
*Assistant Examiner*—William R. Trenor  
*Attorney*—Connolly and Hutz

[54] **PHOTOGRAPHIC VISCOS PROCESSING**  
4 Claims, No Drawings

[52] U.S. Cl..... **96/55,**  
96/62, 96/60, 96/61  
[51] Int. Cl..... **G03c 5/38**  
[50] Field of Search..... 96/50, 60,  
61, 62, 55

**ABSTRACT:** The processing of color photographic films is accelerated and viscous pastes are used for bleaching and fixing by color developing color-photographic images first coating a viscous fixing paste on the developed material and coating on thereafter a viscous bleaching paste. Thereafter the layers of the fixing and bleaching pastes are sprayed off with water and finally the color photographic material is rinsed in water.

## PHOTOGRAPHIC VISCOUS PROCESSING

## PHOTOGRAPHIC VISCOUS PROCESSING

The invention relates to a method of processing exposed color photographic materials, the bleaching and fixing being effected with viscous pastes.

The conventional processing of color-photographic materials comprises, development, bleaching and fixing. It is necessary to rinse the material very thoroughly after color-forming development and before the treatment with the bleaching bath in order to remove substantially all the excess developer. This is necessary, because the surplus developer would itself be oxidized in the bleaching bath and react in the oxidized form with color-couplers to yield an undesirable color fog. Times of 15-20 minutes are necessary for this rinsing, so that this step takes up a large part of the processing time.

The liquid processing baths for bleaching can be replaced by viscous pastes, which contain the necessary processing agents. This paste is applied by conventional devices as a layer on the exposed photographic material. After this treatment, this layer is sprayed off with water. However, when using viscous pastes the long rinsing of the developed material could not be avoided. Up until now the use of such pastes has consequently been restricted to the processing of black-and-white materials and to the developing step when processing color photographic films.

It is among the objects of the invention to accelerate the processing of color-photographic films and to modify the processes so that viscous pastes can also be used for the bleaching and fixing.

We now have found that the time-consuming rinsing between the color development and further processing can be avoided if, in contrast to the conventional sequence a viscous paste which contains the fixing agent is first applied, and then another layer of a viscous paste which contains the bleaching agent is applied. It is highly unexpected no fogging to occur when processing in accordance with the invention, although rinsing only took place for a short time after the development. When using viscous developer pastes, the conventional spraying off of the processing layer with spray nozzles is sufficient.

It is usually desirable to apply the paste containing the bleaching agent immediately after the paste containing the fixing agent has been applied, but the advantages of the method according to the invention are also obtained if there is a brief time interval between the applications.

The processing method according to the invention, makes it possible to shorten successfully the wet processing time for color-photographic negative material by about 50 percent. Similarly the time needed for the wet processing of color-photographic positive and reversal materials can also be considerably shortened.

The conventional arrangements can be used for the application of the processing layers. The layer thicknesses of the pastes containing the fixing agent and the bleaching agent are preferably between 0.1 and 1 mm., advantageously between 0.3 and 0.5 mm. The most suitable thickness of the layer, depends on the concentration of the active substance in the layer, on the photographic material and on the required processing time. The most favorable conditions can be easily established by simple routine tests.

The viscosity of the processing pastes at 50° C. is between 300 and 2000 c.p.s., preferably between 1000 and 1300 c.p.s. It has been found desirable that the viscosity of the bleaching paste be somewhat less than that of the fixing paste. The processing can be carried out at temperatures between 20° and 70° C., preferably between 25° and 40° C.

The processing pastes have the usual compositions. They differ substantially from the conventional baths in that they contain thickeners which produce the pasty consistency. Processing baths which can be used are described in the book by H. Berger "Agfacolor" 1962, or in the work by E. Mutter "Farbphotographie, Theorie und Praxis," Springer Verlag, Vienna 1967. Suitable thickeners for such baths are: cellulose,

derivatives of cellulose such as cellulose ethers, for instance hydroxyethyl cellulose or carboxymethyl cellulose; starch or derivatives thereof; alginates or derivatives thereof, such as salts, carboxymethyl cellulose, synthetic thickeners such as polyvinyl pyrrolidone, polyvinyl alcohol or other water-soluble polymers, for example, the semiamide of the copolymer of methyl vinyl ether and ammonium maleate.

## EXAMPLE

A conventional commercial color-photographic material comprising a red-sensitive layer containing a cyan coupler arranged on a support, a green-sensitive layer containing a magenta coupler and a blue-sensitive layer containing a yellow coupler is exposed and developed with a developer having the following composition:

|    |                                      |         |
|----|--------------------------------------|---------|
| 20 | sodium hexametaphosphate             | 2 g.    |
|    | diethyl paraphenylenediamine sulfate | 2.75 g. |
|    | hydroxylamine sulfate                | 1.2 g.  |
|    | anhydrous sodium sulfite             | 2 g.    |
|    | anhydrous potassium carbonate        | 75 g.   |
|    | potassium bromide                    | 2 g.    |

made up with water to 1 liter; the pH value of the prepared developer is  $11.1 \pm 0.1$ .

The development time is about 7 minutes at 18°-20° C. After the development, water at a temperature of 30° C. is sprayed onto the film with a flat jet nozzle and the film is freed from any adhering water using a conventional suction device.

A viscous fixing bath of the following composition is then applied using an extruder:

|    |                                    |        |
|----|------------------------------------|--------|
| 35 | ammonium thiosulfate               | 150 g. |
|    | anhydrous $\text{Na}_2\text{SO}_3$ | 15 g.  |
|    | $\text{H}_3\text{BO}_3$            | 7.5 g. |
| 40 | glacial acetic acid                | 10 ml. |
|    | hydroxyethyl cellulose             | 11 g.  |
|    | octyl sulfosuccinamide             | 2 ml.  |
|    | pH 4.9                             |        |
|    | viscosity 1110                     |        |

c.p.s.

the layer thickness is 0.6 mm.

Immediately afterwards a bleaching paste having the following composition is applied in a thickness of 0.3 mm. using a second extruder:

|    |                             |        |
|----|-----------------------------|--------|
| 55 | KBr                         | 20 g.  |
|    | potassium ferricyanide      | 100 g. |
|    | hydroxyethyl cellulose      | 11 g.  |
|    | octyl sulfosuccinamide      | 4 ml.  |
|    | pH 6.0-7.5                  |        |
|    | viscosity 1020-10220 c.p.s. |        |

After leaving the film for 4 minutes at 30° C., both layers are rinsed off using a flat jet nozzle and the film is then rinsed in water.

A colored image with satisfactory color reproduction is obtained. The sensitometric testing of the image which is obtained, when compared with an image which has been obtained using the same material, but which has been processed with conventional liquid baths, shows no differences.

If the processing with the viscous pastes is carried out in the usual manner, i.e. first treating the film with the bleaching bath and then with the fixing bath, a colored image is obtained which shows strong color fogging as is usual when no intermediate rinsing with water has been effected. Such images are of no practical value.

What is claimed is:

1. In process for making color-photographic images including the steps of exposing a multilayer color-photographic material to the object to be reproduced, color-developing, and using pastes in bleaching and fixing the exposed material, wherein the layers of the fixing pastes are sprayed off with water and finally the color-photographic material is rinsed in water, the improvement of performing the bleaching and fixing with viscous processing pastes, at a temperature of between 20° and 70° C., whereby the developed material is first coated with layer of the paste containing a thiosulfate fix-

10

ing agent and that layer is overcoated with a second layer containing a ferricyanide bleaching agent.

2. The process of claim 1, wherein the thicknesses of the layer-containing fixing agent and the layer containing the bleaching agent are 0.1-1 mm.

3. The process of claim 1, wherein the viscosity of the processing pastes is between 300 and 2000 c.p.s. at 50° C.

4. The process of claim 1, wherein the processing temperature is between 25° and 40° C.

15

20

25

30

35

40

45

50

55

60

65

70

75

UNITED STATES PATENT OFFICE  
CERTIFICATE OF CORRECTION

Patent No. 3,607,277

Dated SEPTEMBER 21, 1971

Inventor(s) KARL-WILHELM SCHRANZ and ERWIN SCHON

It is certified that error appears in the above-identified patent and that said Letters Patent are hereby corrected as shown below:

Column 2, line 26, "later" should read -- liter -- .  
Column 2, line 39, delete the straight line following "H<sub>3</sub>BO<sub>3</sub>".  
Column 2, line 43, "c.p.s." should follow "1110".  
Column 2, line 58, delete "10220" so line will read --  
viscosity 1020 c.p.s. -- .  
Claim 1, line 5, delete "fixing".

Signed and sealed this 2nd day of May 1972.

(SEAL)

Attest:

EDWARD M. FLETCHER, JR.  
Attesting Officer

ROBERT GOTTSCHALK  
Commissioner of Patents